

## UNITED STATES PATENT OFFICE

REINHOLD REICHMANN, OF BERLIN, GERMANY, ASSIGNOR TO SIEMENS & HALSKE AKTIENGESELLSCHAFT, OF SIEMENSSTADT, NEAR BERLIN, GERMANY, A CORPORATION OF GERMANY

MANUFACTURE OF INSULATING BODIES AND MORE PARTICULARLY OF INSULATORS FOR SPARK PLUGS

No Drawing. Application filed December 2, 1929, Serial No. 411,214, and in Germany October 17, 1928.

My invention relates to improvements in the manufacture of insulating bodies, and more particularly of insulators for spark plugs.

5 It has already been proposed to produce insulating bodies such as insulators for spark plugs and the like, by sintering moulded aluminium oxide. It has, however, been found that the surface of the aluminium oxide sometimes forms a leakage path for the current.

10 My invention relates to a process of sintering aluminium oxide in which this drawback is avoided. My invention consists substantially in carrying out the sintering process in an atmosphere free from reducing carbon-containing gases or vapors. The bodies obtained are similar to marble and have a comparatively smooth surface. The conductivity 15 of the aluminium oxide bodies sintered by the known processes is probably traceable to the fact that aluminium carbide is formed which itself is a conductor of electricity and which under the influence of the humidity of the 20 air decomposes into the likewise conducting aluminium hydroxide.

The sintering of the aluminium oxide bodies is preferably carried out in a vacuum or in a reducing neutral or inert atmosphere. 25 Care must then be taken that no particles of carbon are contained in the furnace which might cause the formation of carbon-containing gases or vapors. If for some reason it is not possible to avoid altogether carbon-containing parts in the furnace, care must be 30 taken to provide an excess of oxygen in the furnace so that carbon-containing gases which may have been generated are oxidized to such an extent that they are no longer able 35 to react on the aluminium oxide. In many cases it is sufficient to pass a current of air through the furnace.

40 Particularly favorable results are obtained if an electric resistance furnace is employed 45 which is equipped with a heating coil of tungsten or any other suitable metal. For the protection of the heating coil a reducing protective gas is preferably employed, for instance a mixture of nitrogen and hydrogen, generally in the proportion of three

parts nitrogen to one part hydrogen. This protective gas is preferably also passed across the body of aluminium oxide to be sintered.

I claim as my invention:

1. The process of producing insulating 55 bodies of aluminium oxide, particularly spark plugs, which consists in sintering the bodies in a chamber free from reducing carbon-containing gases or vapors.

2. The process of producing insulating 60 bodies of aluminium oxide, particularly spark plugs, which consists in sintering the bodies in a vacuum chamber.

3. The process of producing insulating 65 bodies of aluminium oxide, particularly spark plugs, which consists in sintering the bodies in a chamber containing an oxygen-containing atmosphere for maintaining the chamber free from reducing carbon containing gases or vapors.

4. The process of producing insulating 70 bodies of aluminium oxide, particularly spark plugs, which consists in sintering the bodies in an electric furnace free from parts consisting of carbon.

In testimony whereof I affix my signature.  
REINHOLD REICHMANN.

80

85

90

95

100